# EUROPEAN PATENT SPECIFICATION

(11) **EP 2 870 229 B1**
(45) Date of publication and mention of the grant of the patent: **07.08.2019**
(21) Application number: 13730199.0
(22) Date of filing: 14.06.2013
(51) Int. Cl.: C11D 11/02, C11D 1/02, C11D 3/10, C11D 3/37

(54) **PROCESS FOR THE PRODUCTION OF A DETERGENT GRANULE, DETERGENT GRANULE AND DETERGENT COMPOSITION COMPRISING SAID GRANULE**
VERFAHREN ZUR HERSTELLUNG VON WASCHMITTELGRANULAT, WASCHMITTELGRANULAT UND WASCHMITTELZUSAMMENSETZUNG MIT DIESEM GRANULAT
PROCÉDÉ DE PRODUCTION D'UN GRANULE DE DÉTERGENT, GRANULE DE DÉTERGENT ET COMPOSITION DÉTERGENTE COMPRENANT CE GRANULE

(30) Priority: 09.07.2012 EP 12175590
(43) Date of publication of application: 13.05.2015
(73) Proprietor: Unilever N.V., 3013 AL Rotterdam (NL); Unilever PLC, London, Greater London EC4Y 0DY (GB)
(72) Inventor: PACHA, Fakhruddin Esmail, NL-3133 AT Vlaardingen (NL)
(74) Representative: Reijns, Tiemen Geert Pieter
(86) International application number: PCT/EP2013/062387
(87) International publication number: WO 2014/009101

(56) References cited:
- EP-A1- 1 914 297
- EP-A2- 0 221 776

## Description

### TECHNICAL FIELD OF INVENTION

The present invention relates to the field of detergent powders, especially laundry detergent powders, and their production. More in particular, it relates in a first aspect to a process for the production of a detergent granule comprising at least 50% by weight of an anionic surfactant and suitable for use as a granular detergent composition or a component thereof. In a second aspect the invention relates to a detergent granule comprising at least 50% by weight of an anionic surfactant and which is obtainable by said process. In a third aspect the invention to relates detergent compositions comprising such granules.

### BACKGROUND

This invention relates to the production of detergent granules comprising a surfactant system that gives effective washing. In particular, the invention relates to a process to produce such granules by spray-drying an aqueous slurry.

It is well known to prepare granular detergent products or powders by spray-drying of aqueous slurries. Such processes comprise the steps of preparing aqueous slurry comprising from 20 to 60 by weight water, followed by atomising slurry under high pressure to form droplets and then drying these in a counter-current spray-drying tower. Typical tower inlet and outlet temperatures are from 250-400°C and 80-120°C, respectively.

For example, EP-A-1 914 297 discloses a process for the preparation of a spray-dried detergent powder having a bulk density of 426g/l or less, wherein the spray-dried detergent powder comprises an anionic detersive surfactant and from 0% to 10% by weight zeolite builder and from 0% to 10% by weight phosphate builder, and wherein the process comprises the step of:
(a) preparing an aqueous slurry suitable for spray-drying comprising from 30% to 60% by weight water and from 40% to 70% by weight non-aqueous material, wherein the non-aqueous material comprises an inorganic component and an organic component wherein the weight ratio of the inorganic component to organic component is in the range of from 0.3:1 to 5:1; and
(b) spraying the slurry into a spray-drying tower, wherein the temperature of the slurry as it enters the spray-drying tower is in the range of from 65°C to 140°C, and wherein the outlet air temperature of the spray-drying tower is in the range of from 70°C to 120°C and wherein the non-aqueous material comprises anionic surfactant, polymeric carboxylate and carbonate salt.

EP-A-221 776 describes a process for the production of a porous, zero-phosphate powder suitable for use as a base for a granular detergent composition or a component thereof and capable of absorbing and retaining substantial quantities of liquid or liquefiable detergent components in liquid form, which process comprises the steps of (i) preparing an aqueous slurry comprising sodium carbonate, and optionally also comprising sodium sulphate, (ii) drying the slurry to form a powder, the process being characterised in that the total amount of sodium carbonate and (if present) sodium sulphate is at least 20% by weight based on the dried powder, the weight ratio of sodium carbonate to sodium sulphate (when present) in the slurry is at least 0.37:1, and from 0.1 to 60% by weight, based on the total amount of sodium carbonate and (if present) sodium sulphate in the dried powder, of a crystal growth modifier which is a polymeric polycarboxylate is incorporated in the slurry not later than the sodium carbonate, whereby crystal-growth-modified sodium carbonate monohydrate and/or crystal-growth modified Burkeite is or are formed in the slurry. The purpose of the process of EP-A-221 776 is to create a large amount of crystal-growth-modified sodium carbonate monohydrate and/or Burkeite, which are crystalline materials.

These processes can advantageously be used to prepare spray-dried detergent powders having a low bulk density a low content of anionic surfactants. It is difficult, however, to prepare detergent powders having an anionic detergent content of 40% by weight or higher. A further increase in anionic detergent content leads to poor drying rate due to high slurry moisture content of around 40-50%. The high drying temperatures needed for drying off the excess water cost extra energy and may lead to incidences of fire in the tower and/or the dry cyclones. High anionic detergent slurries may also cause overflow and have transportation problems because of aeration and the very high viscosity.

The resulting high anionic detergent powders usually have a low bulk density and are difficult to handle and store and have higher packaging costs.

Moreover, spray-drying is an energy intensive process and it would be interesting from an environmental point of view to improve the current detergent manufacturing technology in this respect. Environmental aspects of detergent manufacturing processes are considered to be important, not only by the manufacturers but also by the consumers who are increasingly interested in the sustainability of our economic activities.

It is therefore a first object of the present invention to provide a more energy efficient process to prepare spray-dried detergent granules having at least 50 wt% of an anionic surfactant that do not have the above-mentioned draw-backs. It particular, the detergent granules should have good powder properties.

It is a further object of the present invention to provide a more energy efficient process to prepare spray-dried (laundry) detergent powders having at least 50 wt% of an anionic surfactant that do not have the above-mentioned draw-backs.

We have now surprisingly found that it is possible to prepare spray-dried (laundry) detergent powders having at least 50 wt% of an anionic surfactant, having an amorphous phase content of more than 60% by weight, by incorporating sodium citrate, up to 5% by weight alkaline silicate, polycarboxylate polymer and sodium carbonate in the slurry. Despite the low level of silicate, the powder properties are excellent.

Thus, these and other objects may be achieved by the process according to the invention for the production of a detergent granule suitable for use as a granular detergent composition or a component thereof, which process comprises the steps of (i) mixing an anionic surfactant precursor with a source of alkali to form a neutralised paste, (ii) adding sodium citrate, up to 5% by weight alkaline silicate, polycarboxylate polymer and sodium carbonate to form a slurry and (iii) spray-drying the obtained slurry to form a detergent granule having an amorphous phase content of more than 60% by weight, preferably more than 70% by weight, whereby the molar ratio of sodium citrate to sodium carbonate is in range of 0.4 to 1.6

### DEFINITION OF THE INVENTION

According to a first aspect of the present invention there is provided a process for the production of a detergent granule comprising at least 50% by weight of an anionic surfactant and suitable for use as a granular detergent composition or a component thereof, which process comprises the steps of (i) mixing an anionic surfactant precursor with a source of alkali to form a neutralised paste, (ii) adding sodium citrate, up to 5% by weight alkaline silicate, polycarboxylate polymer and sodium carbonate to form a slurry and (iii) spray-drying the obtained slurry to form a detergent granule having an amorphous phase content of more than 60% by weight, whereby the molar ratio of the sodium citrate to sodium carbonate is in range of 0.4 to 1.6.

According to a second aspect of the present invention there is provided a spray-dried detergent granule comprising at least 50% by weight of an anionic surfactant, sodium citrate, up to 5% by weight alkaline silicate, polycarboxylate polymer and sodium carbonate and where the detergent granule has an amorphous phase content of more than 60% by weight and the molar ratio of sodium citrate to sodium carbonate is in range of 0.4 to 1.6 and said detergent granule is suitable for use as a granular detergent composition or a component thereof, obtainable by the process according to the invention.

According to a third aspect of the present invention there is provided a detergent composition comprising the granules according to the present invention.

### DETAILED DESCRIPTION OF THE INVENTION

The first aspect of the present invention is a process for the production of a detergent granule comprising at least 50% by weight of an anionic surfactant and suitable for use as a granular detergent composition or a component thereof. Preferably, the detergent granule comprises more than 60 wt% of anionic surfactant.

In a first step of this process, an anionic surfactant precursor is neutralised with a source of alkali to form a surfactant paste. The anionic surfactant precursor is an acid precursor of an anionic non-soap surfactant which, when reacted with a source of alkali, will be neutralised to form a salt of the anionic surfactant.

Anionic surfactant precursors in liquid, pumpable, form are preferred. The anionic surfactant precursor is preferably selected from linear alkyl benzene sulphonic acid, fatty acid and mixtures thereof. Linear alkyl benzene sulphonic acid is also referred to as LAS acid and HLAS. Preferably, the anionic surfactant precursor is LAS acid which yields the corresponding linear alkyl benzene sulphonate (LAS) upon neutralisation. Preferably, the LAS non-soap anionic surfactant has an alkyl chain length of C8-18, more preferably C10-16 and most preferably C12-14.

Soaps formed by the neutralisation of carboxylic or fatty acids may be used as secondary anionic surfactants in admixture with the non-soap anionic surfactants. Preferred carboxylic acids are fatty acids with 12-18 carbon atoms, such as for example fatty acids of coconut oil, palm oil, palm kernel and tallow. The fatty acids may be saturated or unsaturated, branched or straight chain. Mixtures of fatty acids may be used. Fatty acids may be used at levels of up to 30 wt% based on the Anionic surfactant precursor.

The anionic surfactant precursors (or mixture of surfactant precursors) may be used in a partially pre-neutralised form without complete loss of the advantageous effects of the invention. In effect, the surfactant acid is then a mixture of the surfactant acid with neutralised anionic non-soap surfactant.

The anionic surfactant precursors may be added in admixture with other components. Suitable components are neutralised anionic surfactants, for instance the salts of alkyl and/or alkenyl sulphuric acid half-esters (i.e. the sulphation products of primary alcohols) which give alkyl and/or alkenyl sulphates upon neutralisation. Among such non-soap anionic surfactants is primary alcohol sulphate (PAS), especially PAS having a chain length of C10-22, preferably C12-14. Coco PAS is particularly desirable.

Other suitable surfactant acids include alpha-olefin sulphonic acids, internal olefin sulphonic acids, fatty acid ester sulphonic acids and primary sulphonic acids. It is also possible to use combinations of surfactant acids as will be apparent to the skilled person.

Among the other components, in addition to the fatty acids and neutralised anionic surfactant already discussed, the most important additional component that may be added as liquids with the surfactant precursor is nonionic surfactant. This is typically added to the surfactant acid to reduce viscosity to enable it to be added at a lower temperature.

Suitable nonionic surfactants that may be used include the primary and secondary alcohol ethoxylates, especially the C8-C20 aliphatic alcohols ethoxylated with an average of from 1 to 50, preferably 1 to 20, moles ethylene oxide per mole of alcohol, and more especially the primary and secondary aliphatic alcohols ethoxylated with an average of from 1 to 10 moles of ethylene oxide per mole of alcohol. Non-ethoxylated nonionic surfactants include alkyl-polyglycosides, glycerol monoethers, and polyhydroxyamides (glucamide). As discussed already neutralised anionic surfactant may be mixed with the surfactant acid. This can have the advantage of increasing the throughput of the overall process.

Other liquid additives that may be added with the anionic surfactant precursor, or added as separate liquid stream(s), include inorganic acids, such as sulphuric acid, and hydrotropes, such as para toluene sulphonic acid.

The source of alkali that is reacted with the anionic surfactant precursor can be any suitable source of alkali, in liquid or solid form. Examples are aqueous alkali metal hydroxide solutions, preferably sodium hydroxide solutions, or sodium carbonate. Especially preferred are about 50% by weight concentrated aqueous sodium hydroxide solutions. The amount of water should be kept to a minimum, because the water will have to be dried off in the subsequent spray-drying step. On the other hand, it should not be so low that the neutralised surfactant paste is too viscous to handle.

The sodium carbonate may be of any type. Synthetic light soda ash has been found to be especially preferred; natural heavy soda ash is intermediate, while synthetic granular soda ash is the least preferred raw material.

The surfactant paste is preferably prepared in an agitated mixer provided with an open steam coil to heat the mass to a temperature of about 35-40°C. The neutralisation reaction between the anionic surfactant precursor and the source of alkali yields a concentrated surfactant paste, which preferably has a solid content of between 60 to 80% by weight. The heat of neutralisation causes the temperature to rise from about 35-40°C to about 75-80°C, where it is maintained. It is beneficial to allow a few minutes additional time to ensure full neutralization.

In a second step of the process, sodium citrate, up to 5 wt.% alkaline silicate, polycarboxylate polymer and sodium carbonate (Na₂CO₃) are added to the surfactant paste to form a slurry. The order of addition is not believed to be essential.

The polycarboxylic acid used in accordance with the present invention is a monomeric polycarboxylic acid having a relatively low molecular weight of up to 400. It may be may be selected from di-, tri- and tetra-carboxylic acids, whereby tri-carboxylic acids are preferred, especially citric acid. Other possibilities are lactic acid and tartaric acid. The alkali metal salt is preferably a sodium salt. The amount of sodium citrate used is in an amount of 2 to 35% by weight, more preferably from 5 to 25% by weight of the composition.

The composition may further comprise up to 5 wt.% of an alkaline silicate. Alkali metal silicates having a SiO2/M2O ratio, wherein M is sodium ion, of from 1.5 to 3.3, preferably from 1.8 to 2.6, are favourably used, most preferred are amorphous sodium silicates.

The slurry further comprises a polycarboxylate polymer. Preferred polymeric polycarboxylates are used in amounts of from 0.1 to 20 wt%, preferably from 0.2 to 5 wt%, most preferably 1 to 5 wt%, based on the total amount of sodium carbonate. However, higher levels of polymer, for example, up to 30% by weight based on sodium carbonate, may be present in detergent granules of the invention, or full compositions comprising the detergent granules of the invention, for other reasons, for example, building, structuring or anti-redeposition.

The polycarboxylate polymer preferably has a molecular weight of at least 1,000, advantageously from 1,000 to 300,000, in particular from 1,000 to 250,000. Polycarboxylates having a molecular weight from 10,000 to 70,000 are especially preferred. All molecular weights quoted herein are those provided by the manufacturers.

Other preferred polymers are homopolymers and copolymers of acrylic acid or maleic acid. Of special interest are polyacrylates and acrylic acid/maleic acid copolymers. Suitable polymers, which may be used alone or in combination, include the following:
Salts of polyacrylic acid such as sodium polyacrylate, for example Versicol (Trade Mark) E5 E7 and E9 ex Allied Colloids, average molecular weights 4000, 27 000 and 70 000; Narlex (Trade Mark) LD 30 and 34 ex National Adhesives and Resins Ltd, average molecular weights 5000 and 25 000 respectively; and Sokalan (Trade Mark) PA range ex BASF, average molecular weight 250 000; ethylene/maleic acid copolymers, for example, the EMA (Trade Mark) series ex Monsanto; methyl vinyl ether/maleic acid copolymers, for example Gantrez (Trade Mark) AN119 ex GAF Corporation; acrylic acid/maleic acid copolymers, for example, Sokalan (Trade Mark) CP5 ex BASF.

Polyaspartates and polyaspartic acid are advantageously used due to their biodegradability. Polyaspartate is a biopolymer synthesised from L-aspartic acid, a natural amino acid. Due in part to the carboxylate groups, polyaspartate has similar properties to polyacrylate. One preferred type of polyaspartate is thermal polyaspartate or TPA. This has the benefit of being biodegradable to environmentally benign products, such as carbon dioxide and water, which avoids the need for removal of TPA during sewage treatment, and its disposal to landfill. TPA may be made by first heating aspartic acid to temperatures above 180°C to produce polysuccinimide. Then the polysuccinimide is ring opened to form polyaspartate. Because the ring can open in two possible ways, two polymer linkages are observed, an [alpha]-linkage and a [beta]-linkage.

Mixtures of any two or more polymers, if desired, may be used in the process and detergent granule compositions of the invention.

Alkaline silicate and polymer may be pumped into the mixer with increased agitation speed improve the fluidity of total mass.

The slurry further comprises sodium carbonate in an amount of 5-40 % by weight. The sodium carbonate may be of any type. Preferably, the slurry contains less than 10% by weight zeolite builder and less than 10% by weight phosphate builder, even more preferably it is completely free from zeolite builder or phosphate builder.

Optionally, the slurry may comprise sodium carboxymethyl cellulose (SCMC) in an amount of 0.1 to 2.5 % by weight.

In a third next step of the process of the invention, the obtained slurry is spray-dried to form a granule having an amorphous phase content of more than 60% by weight, preferably more than 70% by weight, whereby the molar ratio of the sodium citrate to sodium carbonate is in range of 0.4 to 1.6. Typical tower inlet and outlet temperatures of the spray-drying process are from 250-400°C and 80-120°C, respectively.

### The detergent granule

A second aspect of the present invention is a spray-dried detergent granule comprising at least 50% by weight of an anionic surfactant and suitable for use as a granular detergent composition or a component thereof. The granules has a relatively high specific surface area which makes them suitable as carrier for absorbing liquid components such as nonionic surfactants or nonionic surfactant/ fatty acid blends.

The granule according to the invention comprises:
(i) at least 50% by weight anionic surfactant, soap and mixtures thereof,
(ii) sodium citrate,
(iii) up to 5 wt% alkaline silicate,
(iv) polycarboxylate polymer,
   and sodium carbonate,
   the detergent granule has an amorphous phase content of more than 60% by weight
   the molar ratio of sodium citrate to sodium carbonate is in the range of 0.4 to 1.6 obtainable by the process of the present invention.
Preferably, the alkali metal salt of a non-soap detergent is linear alkylbenzene sulphonate (LAS).

The spray-dried detergent granule of the invention is a particulate solid with a bulk density in the range of 250 to 500 g/litre. The particle size distribution is generally such that at least 50 wt%, preferably at least 70 wt% and more preferably at least 85 wt%, of particles are smaller than 1700 microns, and the level of fines is low. No further treatment has generally been found to be necessary to remove either oversize particles or fines.

The spray-dried detergent granule is further characterised by its specific surface area, measured by nitrogen adsorption. The specific surface area ("SSA") of the granules is measured by nitrogen absorption according to ASTM D 3663-78 standard based upon the Brunauer, Emmett, and Teller (BET) method described in J. Am. Chem. Soc. 60, 309 (1938). We used a Gemini Model 2360 surface area analyzer (available from Micromeritics Instrument Corp. of Norcross, Ga.). The spray-dried detergent granule has a specific surface area (SSA) of 5 m²/g or greater, preferably 8 m²/g or greater, even more preferably 10 m²/g or greater.

The obtained granule generally has excellent flow properties, low compressibility and little tendency towards caking. The particulate detergent granules that are the direct result of the spray-drying process have an anionic surfactant content of at least 50wt%. There is no need for a granulation aid such as zeolite, although it is possible to use them. It is possible to achieve exceptionally high levels of anionic surfactant in the granule. For example, greater than 50 wt%, or over 50 wt% anionic surfactant may be incorporated into the detergent granule. It is preferred for the anionic surfactant to comprise less than 10 wt% soap, based on the total anionic surfactant in the detergent granule.

The detergent granules may also comprise water in an amount of 0 to 8% and preferably 0 to 4% by weight of the granules. The detergent granules obtained from the process are storage stable at high levels of humidity. Thus, they can be used in a wide range of detergent products.

Desirably the detergent granules have an aspect ratio not in excess of two and more preferably are generally spherical in order to reduce segregation from other particles in a formulated powder detergent composition and to enhance the visual appearance of the powder.

The presence of the amorphous phase can be detected using X-ray diffraction techniques that are known in the art. X-ray diffraction (XRD) is a non destructive analytical method for measuring characteristic diffraction angles and intensities from periodically ordered matter (crystalline material). Intensity and spatial distributions of the scattered X-rays form a specific diffraction pattern, which is the "fingerprint" of the sample and can be used for qualitative and quantitative evaluation, d-value calculation, the determination of crystallite size and defects by the peak shape and polymorphism.

### The detergent composition

A third aspect of the present invention is a detergent composition, especially a laundry detergent composition, comprising the granules according to the present invention.

The spray-dried detergent granules of the present invention may be used as such, but they may also be supplemented with other detergent ingredients, components or additives to form a complete detergent composition. The detergent granules may be admixed with anything normally used in detergent formulations. They may be dry blended with solid materials and they may advantageously have further liquids added into them, using their spare liquid carrying capacity. It is especially advantageous to add conventional, or even higher than conventional, levels of perfume this way.

Other types of non-soap surfactant, for example, cationic, zwitterionic, amphoteric or semipolar surfactants, may also be used with the granules if desired. Many suitable detergent-active compounds are available and are fully described in the literature, for example, in "Surface-Active Agents and Detergents", Volumes I and II, by Schwartz, Perry and Berch.

Soap may also be present, to provide foam control and additional detergency and builder power. The fully formulated composition may comprise up to 8 wt% soap. The total amount of surfactant present in the fully formulated detergent composition is suitably from to 15 to 70 wt%, although amounts outside this range may be employed as desired.

The fully formulated detergent compositions including the detergent granules prepared by the process of the invention may contain conventional amounts of other detergent ingredients, for example, bleaches, enzymes (preferably protease, lipase, amylase and/or cellulase), lather boosters or lather controllers as appropriate, anti-redeposition agents such as cellulosic polymers; anti-incrustation agents, perfumes, dyes, shading dyes, fluorescers, sodium silicate; corrosion inhibitors including silicates; inorganic salts such as sodium sulphate, coloured speckles; foam controllers; and fabric softening compounds. It is especially preferred if the fully formulated detergent composition contains TAED/percarbonate as bleaching system.

The detergent granule may if desired be mixed with other organic or inorganic builders, typically supplied in the form of granules of either pure builder or mixtures of builder and other ingredients. Especially preferred organic builders are acrylic polymers, more especially acrylic/maleic copolymers, suitably used in amounts of from 0.5 to 15 wt%, preferably from 1 to 10wt%.

The detergent granules of the present invention are hereinafter called a base powder. They may be mixed with another powder obtained from any conventional detergent production process including spray drying or non spray drying processes. As the detergent granules produced by the present invention may be admixed with such other powders, a significant degree of formulation flexibility is obtained and the level of active material in the fully formulated composition may be very high without an unnecessary increase in builder levels.

The detergent granules may typically form from 30 to 100 wt% of a final fully formulated detergent composition. Typically, the fully formulated detergent composition incorporating the detergent granules produced by the process of the invention may comprise from 15 to 60 wt%, preferably 20 to 50 wt% of anionic surfactant, this anionic surfactant being derived wholly or in part from the granular product of the spray-drying process. In addition, the fully formulated detergent composition may comprise from 0 to 35 wt% of nonionic surfactant, and from 0 to 5 wt% of fatty acid soap.

Fully formulated detergent compositions, comprising other ingredients and the detergent granules produced according to the invention preferably have a bulk density of about 250 to 750 g/litre, more preferably at least 350 g/litre.

Fully formulated detergent compositions may also include other solid ingredients desired for inclusion in the detergent powder, for example, fluorescers; polycarboxylate polymers; antiredeposition agents such as, for example, sodium carboxymethyl cellulose (SCMC); or fillers such as sodium sulphate, diatomaceous earth, calcite, kaolin or bentonite.

If desired, solid particulate surfactants, for example, alkylbenzene sulphonate and/or alkyl sulphate in powder form, may form part of the solids charge to the mixer to further increase the activity level of surfactant in the granule, however it is preferred to produce all the anionic surfactant by spray-drying.

The process is generally not sensitive to the type of mixer used, provided intensive mixing is applied. We have found that to obtain the full advantages of the invention the use of a mixer with a chopping action may be advantageous.

Preferably, the mixing is carried out in a mixer having and using both a stirring action and a cutting action, most preferably these actions will be separately usable, as described below. The cutting action is the preferred chopping action. This may be advantageously achieved by the choice of mixer to be a high-speed mixer/granulator having both a stirring action and a cutting action. Preferably, the high-speed mixer/granulator has rotatable stirrer and cutter elements that can be operated independently of one another, and at separately changeable or variable speeds.

Such a mixer is capable of combining a high-energy stirring input with a cutting action, but can also be used to provide other, gentler stirring regimes with or without the cutter in operation. A Lödige mixer is preferred, vertical or horizontal axis cutters are desirable for high anionic loading. Also preferred are mixers of the Fukae FS-G type manufactured by Fukae Powtech Co Ltd., Japan; this apparatus is essentially in the form of a bowl-shaped vessel accessible via a top port, provided near its base with a stirrer having a substantially vertical axis, and a cutter positioned on a side wall. The stirrer and cutter may be operated independently of one another, and at separately variable speeds. The vessel can be cooled.

Other mixers believed to be suitable for use in the process of the invention are the Fuji (Trade Mark) VG-C series ex Fuji Sangyo Co., Japan; and the Roto (Trade Mark) ex Zanchetta & Co srl, Italy.

Yet another mixer found to be suitable for use in the process of the invention is the Lödige (Trade Mark) FM series batch mixer ex Morton Machine Co. Ltd., Scotland. This differs from the mixers mentioned above in that its stirrer has a horizontal axis. Z blade and sigma mixers (Winkworth machinery limited) are suitable mixers having a chopping action.

The invention will now be further described with reference to the following non-limiting examples. In the examples, the Bulk Density (BD), Dynamic Flow Rate (DFR) and Unconfined Compression Test (UCT) are measured according to the following known test protocol.

### Bulk density (BD)

The bulk density properties in the present specification are measured by a method according to JIS K 3362.

### Dynamic flow rate (DFR)

This is also called flow-rate. Powder flow may be quantified by means of the dynamic flow rate (DFR), in ml/s, measured by means of the following procedure. The apparatus used consists of a cylindrical glass tube having an internal diameter of 40 mm and a length of 600 mm. The tube is securely clamped in a position such that its longitudinal axis is vertical. Its lower end is terminated by means of a smooth cone of polyvinyl chloride having an internal angle of 15° and a lower outlet orifice of diameter 22.5 mm. A first beam sensor is positioned 150 mm above the outlet, and a second beam sensor is positioned 250 mm above the first sensor.

To determine the dynamic flow rate of a powder sample, the outlet orifice is temporarily closed, for example, by covering with a piece of card, and powder is poured through a funnel into the top of the cylinder until the powder level is about 10 cm higher than the upper sensor; a spacer between the funnel and the tube ensures that filling is uniform. The outlet is then opened and the time t (seconds) taken for the powder level to fall from the upper sensor to the lower sensor is measured electronically. The measurement is normally repeated two or three times and an average value taken. If V is the volume (ml) of the tube between the upper and lower sensors, the dynamic flow rate DFR (ml/s) is given by the following equation: $DFR = \frac{V}{t} ml/s$

### Unconfined Compression Test (UCT)

In this test, freshly produced powder is compressed into a compact and the force required to break the compact is measured. The powder is loaded into a cylinder and the surface levelled. A 50 g plastic disc is placed on top of the powder and a 10 kg weighted plunger is placed slowly on top of the disc and allowed to remain in position for 2 minutes. The weight and plunger are then removed and the cylinder removed carefully from the powder to leave a free-standing cylinder of powder with the 50g plastic disc on top of it. If the compact is unbroken, a second 50 g plastic disc is placed on top of the first and left for approximately ten seconds. Then if the compact is still unbroken a 100 g disc is added to the plastic discs and left for ten seconds. The weight is then increased in 0.25 kg increments at 10 second intervals until the compact collapses. The total weight (w) needed to effect collapse is noted.

The cohesiveness of a powder is classified by the weight (w) as follows:
w < 1.0 kg Good flowing
1.0 kg < w < 2.0 kg Moderate flowing.
2.0 kg < w < 5.0 kg Cohesive.
5.0 kg < w Very cohesive.

### EXAMPLES

Examples 1-7 (NB Ex. 2 is not illustrative of the invention as claimed) 2,300 kg of an aqueous slurry was prepared in an agitated vessel provided with an open steam coil to heat the mass, involving the following steps.

A charge made of clean water (563 kg) and caustic soda solution (197 kg) of 50% purity was dosed to an agitated vessel, provided with an open steam coil and a Lightnin A320 impeller. The charge was heated to a temperature of 35-40°C and subsequently, 1.9 kg of Tinopal CBSX was mixed until fully dissolved. Following this step, pre-weighed quantity (753 kg) of commercial grade of sulphonic acid was dosed gradually over a period of 3-4 minutes with continuous agitation to form neutralized paste. Additional time of 2 minutes was allowed to ensure that the neutralization was complete. 342 kg of sodium citrate (di-hydrate) and 45 kg of Lutensol EO7 were sequentially added to form uniform mass. Preheated alkaline silicate (50 kg) and copolymer (150kg) were pumped into the mixer with increased agitation speed so that it improved fluidity of total mass. At this stage, it may be preferred to maintain temperature at 75-80°C by use of steam in open coil. Following this step, steam valve was shut off and 199 kg sodium carbonate along with 16.1 kg SCMC were dosed via screw conveyor adjusted to dose over a period of 2-3 minutes and agitator speed set to 70-75 rpm. When dosing solids, they fell close to the agitator blades to prevent build up on the wall or lump formation. A final mixing step was allowed for another 2 minutes and then the mixed mass at 80°C was discharged to the holding tank for subsequent operation in the spray drying tower.

In all examples, the above charge sheet was calculated for various formulations and used for making slurries. The slurries were transported by a low pressure pump, Reitz mill/magnetic separator and then to the high pressure pump. The slurry was sprayed in a 2.5 meter dia spray drier by use of two spraying system nozzles to achieve desired throughput rate of 1000-1100 kg/hr of slurry at pressures of 25-28 bars. The tower was supplied by hot air maintained at temperatures of 270-290°C in counter current mode and dried powder was collected at the bottom of tower. Powder moisture content was controlled in the range of 3-4% and minor variations in air inlet temperature were required to maintain steady state conditions.

The powder properties were measured as given below and a layering agent like Aerosil was applied to achieve good storage stable product.

The following powder properties were measured for the base powders with and without Nonionics EO7:

| Sample Code | | |
|---|---|---|
| | **Example 3** | **Example 4** |
| AD level | 55 | 52 |
| NI 7 EO | 0 | 3 |
| BD (g/l) | 423 | 311 |
| DFR (ml/sec) | 102 | 96 |
| UCT (gm) | 200 | 450 |
| VCT (%) | 10 | 11 |
| PMC (%) | 3.1 | 2.69 |

| PSD (micron) | | |
|---|---|---|
| 1400 | 0.5 | 1.00 |
| 1000 | 0.58 | 3.47 |
| 710 | 3.02 | 11.21 |
| 500 | 16.61 | 26.47 |
| 250 | 47.75 | 35.87 |
| 180 | 13.92 | 10.18 |
| 120 | 9.52 | 5.9 |
| 0 | 8.1 | 5.9 |
| Total (gm) | 100.0 | 100 |

The powder properties were examined as given below and additional nonionic / fatty acid blend was sprayed onto the tower base powder (indicated by % Active loaded) to give a detergent product having excellent powder properties.

The base powders of Examples 1-7 were also examined for presence of crystalline phases. Using the D8 Discover ex Bruker-AXS machine, the d-values of the diffraction lines of the samples were obtained and from them the crystalline compounds were identified.

### Materials and methods:

| | 2θ (5 - 55°) |
|---|---|
| Theta 1 | 4.500 |
| Theta 2 | 10.000/25.000/40.000 |
| Phi (only transmission) | - |
| Detector Bias (kV / mA) | 40 / 40 |
| Time (sec) | 150 |
| Collimator (mm) | 0.3 (monocap) |
| Detector distance (cm) | 25 |
| Tube Anode | Cu |
| Used SLM file | Detergent.slm |

The presence of crystalline compounds in base powders are given in the table below:

| Example | 1 | 2 | 3 | 4 | 5 | 6 | 7 |
|---|---|---|---|---|---|---|---|
| **XRD diffraction** | | | | | | | |
| Amorphous -XRD (wt%) | 79.0 | 81.0 | 78.0 | 79.0 | 86.0 | 87.0 | 81.0 |
| Sodium carbonate, anhydrous | 21 | 19 | 22 | 21 | 14 | 13 | 19 |

It follows from these XRD data that these base powders contain mostly amorphous phases and present sodium carbonate as anhydrous crystals.

## Claims

1. Process for the production of a detergent granule comprising at least 50% by weight of an anionic surfactant and suitable for use as a granular detergent composition or a component thereof, which process comprises the steps of
(i) mixing an anionic surfactant precursor with a source of alkali to form a neutralised paste,
(ii) adding sodium citrate, up to 5% by weight alkaline silicate, polycarboxylate polymer and sodium carbonate to form a slurry and
(iii) spray-drying the obtained slurry to form a detergent granule having an amorphous phase content of more than 60% by weight,
whereby the molar ratio of sodium citrate to sodium carbonate is in range of 0.4 to 1.6.

2. Process according to claim 1, wherein the anionic surfactant precursor is selected from Linear Alkylbenzene Sulphonic (LAS) acid, fatty acid and mixtures thereof.

3. Process according to any preceding claim in which the slurry comprises 1 to 3% by weight amorphous sodium silicate.

4. Process according to claim 3, in which the polymer is selected from acrylic acid homopolymers, acrylic acid/maleic acid copolymers, and acrylic phosphinates.

5. Process according to claim 4, **characterised in that** the polymer is sodium polyacrylate.

6. Process according to claim 5, **characterised in that** the polymeric polycarboxylate has a molecular weight within the range of from 1,000 to 250,000, preferably within the range of from 3,000 to 100,000.

7. Process according to any preceding claim, in which the slurry comprises nonionic surfactant.

8. Process according to any preceding claim, in which the slurry comprises sodium carboxy methyl cellulose.

9. Process according to any preceding claim in which the granule is **characterised by** having a specific surface area of 5 m²/g or greater, preferably 8 m²/g or greater, even more preferably 10 m²/g or greater.

10. A spray-dried detergent granule comprising at least 50% by weight of an anionic surfactant, sodium citrate, up to 5% by weight alkaline silicate, polycarboxylate polymer and sodium carbonate and where the detergent granule has an amorphous phase content of more than 60% by weight and the molar ratio of sodium citrate to sodium carbonate is in range of 0.4 to 1.6 and said detergent granule is suitable for use as a granular detergent composition or a component thereof, obtainable by the process according to any preceding claim.

11. Detergent granule according to claim 10, **characterised by** having a specific surface area of 5 m²/g or greater, preferably 8 m²/g or greater, even more preferably 10 m²/g or greater.

12. Detergent composition comprising the granules according to any one of claims 10 and 11.

13. Detergent composition according to claim 12, further comprising soap and/or nonionic surfactant.

14. Detergent composition according to any one of claims 12 and 13, further comprising a bleach system such as TAED/percarbonate.

15. Detergent composition according to any one of claims 12-14, further comprising fluorescer, preferably at a level of 0.05 to 0.5 wt%.

## Patentansprüche

1. Verfahren zur Herstellung eines Waschmittelgranulats, umfassend mindestens 50 Gewichts-% eines anionischen Tensids und geeignet zur Verwendung als granulare Waschmittelzusammensetzung oder als Bestandteil davon, wobei das Verfahren die Schritte umfasst:
(i) Mischen der Vorstufe eines anionischen Tensids mit einer Alkaliquelle, um eine neutralisierte Paste zu bilden,
(ii) Zugeben von Natriumcitrat, bis zu 5 Gewichts-% alkalisches Silicat, Polycarboxylatpolymer und Natriumcarbonat, um eine Aufschlämmung zu bilden, und
(iii) Sprühtrocknen der erhaltenen Aufschlämmung, um ein Waschmittelgranulat zu bilden, das einen Gehalt an amorpher Phase von mehr als 60 Gewichts-% aufweist,
wobei das Molverhältnis von Natriumcitrat zu Natriumcarbonat in dem Bereich von 0,4 bis 1,6 liegt.

2. Verfahren nach Anspruch 1, wobei die Vorstufe des anionischen Tensids unter linearer Alkylbenzolsulphon(LAS)säure, Fettsäure und Mischungen davon ausgewählt wird.

3. Verfahren nach irgendeinem vorhergehenden Anspruch, in welchem die Aufschlämmung 1 bis 3 Gewichts-% amorphes Natriumsilicat umfasst.

4. Verfahren nach Anspruch 3, in welchem das Polymer unter Acrylsäure-Homopolymeren, Acrylsäure/Maleinsäure-Copolymeren und Acrylphosphinaten ausgewählt wird.

5. Verfahren nach Anspruch 4, **dadurch gekennzeichnet, dass** das Polymer Natriumpolyacrylat ist.

6. Verfahren nach Anspruch 5, **dadurch gekennzeichnet, dass** das polymere Polycarboxylat ein Molekulargewicht innerhalb des Bereichs von 1.000 bis 250.000, vorzugsweise innerhalb des Bereichs von 3.000 bis 100.000, aufweist.

7. Verfahren nach einem vorhergehenden Anspruch, in welchem die Aufschlämmung nichtionisches Tensid umfasst.

8. Verfahren nach einem vorhergehenden Anspruch, in welchem die Aufschlämmung Natriumcarboxymethylcellulose umfasst.

9. Verfahren nach irgendeinem vorhergehenden Anspruch, in welchem das Granulat **dadurch gekennzeichnet ist, dass** es eine spezifische Oberfläche von 5 m²/g oder größer, vorzugsweise von 8 m²/g oder größer, sogar bevorzugter von 10 m²/g oder größer, aufweist.

10. Sprühgetrocknetes Waschmittelgranulat, umfassend mindestens 50 Gewichts-% eines anionischen Tensids, Natriumcitrat, bis zu 5 Gewichts-% alkalisches Silicat, Polycarboxylatpolymer und Natriumcarbonat und wobei das Waschmittelgranulat einen Gehalt an amorpher Phase von mehr als 60 Gewichts-% aufweist und das Molverhältnis von Natriumcitrat zu Natriumcarbonat in dem Bereich von 0,4 bis 1,6 liegt und das Waschmittelgranulat zur Verwendung als granulare Waschmittelzusammensetzung oder ein Bestandteil davon geeignet ist, erhältlich durch das Verfahren nach irgendeinem vorhergehenden Anspruch.

11. Waschmittelgranulat nach Anspruch 10, **gekennzeichnet durch** eine spezifische Oberfläche von 5 m²/g oder größer, vorzugsweise von 8 m²/g oder größer, sogar bevorzugter von 10 m²/g oder größer.

12. Waschmittelzusammensetzung, umfassend das Granulat nach irgendeinem der Ansprüche 10 und 11.

13. Waschmittelzusammensetzung nach Anspruch 12, ferner umfassend Seife und/oder nichtionisches Tensid.

14. Waschmittelzusammensetzung nach irgendeinem der Ansprüche 12 und 13, ferner umfassend ein Bleichsystem, wie zum Beispiel TAED/Percarbonat.

15. Waschmittelzusammensetzung nach irgendeinem der Ansprüche 12-14, ferner umfassend ein Fluoreszenzmittel, vorzugsweise in einem Anteil von 0,05 bis 0,5 Gew.-%.

## Revendications

1. Procédé pour la production d'un granulé de détergent comprenant au moins 50 % en masse d'un tensioactif anionique et utilisable comme une composition de détergent granulaire ou un constituant de celle-ci, lequel procédé comprend les étapes de :
(i) mélange d'un précurseur de tensioactif anionique avec une source d'alcali pour former une pâte neutralisée,
(ii) addition de citrate de sodium, jusqu'à 5 % en masse de silicate alcalin, de polymère de polycarboxylate et de carbonate de sodium pour former une suspension et
(iii) séchage par pulvérisation de la suspension obtenue pour former un granulé de détergent ayant une teneur en phase amorphe supérieure à 60 % en masse,
sur quoi le rapport molaire de citrate de sodium à carbonate de sodium se trouve dans l'intervalle de 0,4 à 1,6.

2. Procédé selon la revendication 1, dans lequel le précurseur de tensioactif anionique est choisi parmi un acide alkylbenzène sulfonique linéaire (LAS), un acide gras et des mélanges de ceux-ci.

3. Procédé selon l'une quelconque des revendications précédentes, dans lequel la suspension comprend de 1 à 3 % en masse de silicate de sodium amorphe.

4. Procédé selon la revendication 3, dans lequel le polymère est choisi parmi des homopolymères d'acide acrylique, des copolymères d'acide acrylique/acide maléique, et des phosphinates acryliques.

5. Procédé selon la revendication 4, **caractérisé en ce que** le polymère est le polyacrylate de sodium.

6. Procédé selon la revendication 5, **caractérisé en ce que** le polycarboxylate polymère présente une masse moléculaire dans l'intervalle de 1 000 à 250 000, de préférence dans l'intervalle de 3 000 à 100 000.

7. Procédé selon l'une quelconque des revendications précédentes, dans lequel la suspension comprend un tensioactif non ionique.

8. Procédé selon l'une quelconque des revendications précédentes, dans lequel la suspension comprend de la carboxyméthylcellulose de sodium.

9. Procédé selon l'une quelconque des revendications précédentes, dans lequel le granulé est caractérisé en présentant une surface spécifique de 5 m²/g ou supérieure, de préférence de 8 m²/g ou supérieure, encore mieux de 10 m²/g ou supérieure.

10. Granulé de détergent séché par pulvérisation comprenant au moins 50 % en masse d'un tensioactif anionique, du citrate de sodium, jusqu'à 5 % en masse de silicate alcalin, un polymère de polycarboxylate et du carbonate de sodium et où le granulé de détergent présente une teneur en phase amorphe supérieure à 60 % en masse et le rapport molaire de citrate de sodium à carbonate de sodium se trouve dans l'intervalle de 0,4 à 1,6 et ledit granulé de détergent est utilisable comme une composition de détergent granulaire ou un constituant de celle-ci, pouvant être obtenu par le procédé selon l'une quelconque des revendications précédentes.

11. Granulé de détergent selon la revendication 10, **caractérisé en ce qu'**il présente une surface spécifique de 5 m²/g ou supérieure, de préférence de 8 m²/g ou supérieure, encore mieux de 10 m²/g ou supérieure.

12. Composition de détergent comprenant les granulés selon l'une quelconque des revendications 10 et 11.

13. Composition de détergent selon la revendication 12, comprenant de plus du savon et/ou un tensioactif non ionique.

14. Composition de détergent selon l'une quelconque des revendications 12 et 13, comprenant de plus un système de blanchiment, tel que TAED/percarbonate.

15. Composition de détergent selon l'une quelconque des revendications 12-14, comprenant de plus un fluorescent, de préférence à une teneur de 0,05 à 0,5 % en masse.
